

## UNITED STATES PATENT OFFICE.

CHARLES R. FELIX, OF HATFIELD, PENNSYLVANIA.

## COMPOSITION FOR TREATING PRODUCTS OF FIBER AND METHOD OF MAKING SAME.

No Drawing.

Application filed March 6, 1925. Serial No. 13,496.

My invention relates to compositions suitable for the treatment of paper products or paper stock for the purpose of stiffening and rendering the same fire-proof; and also for 5 the purpose of treating both cotton and woolen fabrics for the purpose of rendering the same fire-proof.

It is desireable that pies and the like may be baked upon pie plates of cellulosic material such as ordinary paper pulp, but it has not heretofore been practical to do so because of the incapacity of plates formed and consisting of such material to withstand the temperature required for the baking of pies 10 and the like.

It is also desirable that fabrics, such as cotton, woolen and the like, adapted for certain uses, such for example as curtains and the like, should be rendered fire-proof, 20 but thus far, so far as I am aware, no practical means has been found by which this result might be obtained.

The general object, therefore, of my invention is to provide a composition which is 25 adapted to be employed for the treatment of products of the character indicated for rendering the same fire-proof.

It is also an object of the invention to 30 provide a novel composition which is adapted particularly for the treatment of sheets of cellulosic or other like material for the purpose of stiffening and rendering the same fire-proof.

It is another object of the invention to 35 provide a composition consisting of ingredients which cooperate in such manner that the composition remains and continues as a liquid during the process of using the same at the temperature necessary to the successful 40 employment thereof.

Other objects and advantages of the invention will be pointed out in the detailed description thereof which follows or will be apparent from said description. In describing 45 the invention in detail I shall refer first to the specific composition which I have found to be best adapted for use in the treatment of sheet cellulosic material made from ordinary paper pulp. This material 50 may consist either of pulp produced from wood of finer grades, or pulp produced from rags and the like. Preferably, the best grade of pulp should be employed whether it be produced from wood or from rags.

55 In the production of a composition embodying my invention which is adapted for

the treatment of sheet material of the character indicated I heat about two gallons of water to a temperature of from one hundred and eighty to two hundred degrees Fahrenheit and add thereto seventy-two grams of sodium carbonate and stir or otherwise agitate the same for about five minutes to cause the carbonate to thoroughly and completely dissolve. The temperature of the solution 60 at the end of such period of five minutes probably would be about one hundred and sixty degrees Fahrenheit. Into the solution thus formed one quart of sodium silicate at forty degrees Baumé is then introduced 65 slowly, preferably in a small stream. Simultaneously with the introduction of the sodium silicate into the solution of sodium carbonate and water the mass is stirred and such stirring is continued until the solution 70 becomes clear. Thereafter forty-six grams of tungstate of soda is introduced slowly into the composition or solution thus formed. The tungstate of soda is in the form of a powder and is sprinkled into the said solution 75 and the mass is stirred for from five to ten minutes until the said tungstate of soda is completely dissolved at which time the mass or composition should be clear.

It should be understood that if a larger 80 volume of the mass or composition is desired the quantities of water and the various ingredients or substances added thereto should be increased to the extent necessary to produce the quantity of the composition desired. 85

In the use of the composition which is in liquid form it is placed in a tank and maintained at a temperature of about one hundred and ninety degrees Fahrenheit. The web of paper is then caused to travel through the 90 said tank and each portion thereof is held submerged within the composition in the tank for about twenty seconds. Any suitable known mechanism for causing the web of paper to travel through the tank may be 95 employed. Said treatment not only results in stiffening the sheet, but also in rendering the same fire-proof. After the paper in the form of a web and of a thickness suitable for the manufacture of pie plates, kitchen 100 utensils and plates of other character has been subjected to the action of the composition portions are cut or stamped therefrom and molded to the shape desired. Instead of treating the material in the form of a web the articles such as pie plates and the like may be previously formed and treated, 105 110

but it is more expedient and more economical to treat the material in the form of a web and thereafter stamp out portions thereof and press or mold the same to the shape desired.

The composition as above described is not entirely suitable for the treatment of fabrics of the character already indicated for rendering the same fire-proof because it renders them too stiff for satisfactory use.

I have, however, provided a composition slightly different from that above described which is well adapted for the treatment of fabrics of the character of those already indicated to render the same fire-proof without, however, stiffening them to such an extent as to make them unsuitable for the uses to which such fabrics are usually put. In the making of the composition now under consideration I first heat about two gallons of water to a temperature of from one hundred and eighty to two hundred degrees Fahrenheit and add thereto about fourteen and two-tenths grams of boric acid which is completely dissolved in the water. By the time that such solution is formed the temperature of the water has probably fallen to about one hundred and sixty degrees Fahrenheit. Thereafter one hundred and fifty cubic centimeters of sodium silicate at forty degrees Baumé are added in the form of a small stream. Simultaneously with the addition of the sodium silicate the solution of water and boric acid is stirred and such stirring is continued until the solution becomes entirely clear. To the solution thus formed forty-six grams of tungstate of soda are added slowly. The tungstate of soda is sprinkled into or onto the said solution and the whole mass stirred for from five to ten minutes until the tungstate of soda is completely dissolved and until the mass or composition becomes entirely clear. The compound formed of the ingredients in substantially the quantities and proportions as last described is suitable for the treatment of fabrics such as cotton, woolen and the like for rendering the same fire-proof. If, however, it is desired that a composition of the character of that last described shall be used for the treatment of sheets of cellulosic material of the character as above described to be used in the manufacture of pie plates and other analogous articles the amount of boric acid should be increased to approximately twenty-eight and eight-tenths grams. When the quantity of the boric acid is thus increased a composition is produced which when employed for treatment of sheets of cellulosic material not only renders the same fire-proof but also stiffens the same to such an extent that they are well adapted for use in the manufacture of pie plates, kitchen utensils, plates and other products of analogous character.

It will be understood that the quantities and the proportions of the various ingredients employed in the manufacture of the compositions above described may be varied within practical limits without departing from the spirit and the scope of my invention. In other words, it is to be understood that my invention is not limited to the exact proportions and quantities of ingredients as hereinabove set forth.

When any one of the compositions is being employed for the treatment of products of the character indicated it is necessary that it shall be and remain in liquid form at the temperature, one hundred and ninety degrees Fahrenheit, at which it is employed and during the period of its employment or use. In the first of the compositions described the sodium carbonate operates to prevent gelatinization during use while in the case of the other compositions mentioned the boric acid acts to prevent gelatinization of the compositions. Accordingly, therefore, I regard each of these ingredients as a stabilizing agent because if they were not present in the composition as described, each of the compositions in use would be converted into a gelatinous mass.

It will be seen that by my invention I have provided compositions by the employment of which in the treatment of products of the character indicated such products may be fundamentally altered whereby they possess certain attributes of very great value which ordinarily and generally are foreign thereto.

By the employment of the first composition described to treat paper products to render the same satisfactory for use in the manufacture of pie plates and the like such plates and the like may be very economically produced. Such paper products may also be employed not only for the manufacture of pie plates, etc., but also for the manufacture of cups,—in fact for the manufacture of anything for which such products may be found to be suitable. Like advantages also result from the use of the compositions in which boric acid is employed for the treatment of fabrics of the character indicated and also paper products.

Having thus described my invention what I claim and desire to secure by Letters Patent is:

1. A composition for the treatment of products of cellulosic sheet material consisting of approximately one quart of liquid silicate of soda of a density of about 40° Baumé, approximately forty-six grams of tungstate of soda and a stabilizing substance in requisite quantity all in solution in approximately two gallons of water.

2. A composition for the treatment of products of cellulosic sheet material consisting of sodium carbonate, silicate of soda and

tungstate of soda in the proportions of one quart of liquid silicate of soda of a density of about 40° Bé., forty-six grams of tungstate of soda and seventy-two grams of 5 sodium carbonate to two gallons more or less of water, the said first named ingredients being dissolved in said water.

3. The method of producing a composition which is adapted for the treatment of products of organic material to render the same fire-proof which consists in heating approximately two gallons of water to a temperature of from one hundred and eighty to hundred degrees Fahrenheit, dissolving therein 10 approximately one quart of silicate of soda and approximately forty-six grams of tungstate of soda and thereafter adding to the solution thus formed a soluble chemical material which operates as a stabilizing agent to 15 prevent gelatinization of the composition during its use in the treatment of such products.

4. The method of producing a composition which is adapted for the treatment of products of organic material to render the same fire-proof which consists in heating a suitable volume of water to a temperature of from one hundred and eighty to two hundred degrees Fahrenheit and adding thereto 20 sodium carbonate and stirring until the latter is completely dissolved, during which period the temperature of the water is re-

duced to about one hundred and sixty degrees Fahrenheit, then slowly introducing into the sodium carbonate solution silicate 35 of soda, simultaneously stirring the same and continuing to stir the same until the solution becomes clear and thereafter adding tungstate of soda slowly and stirring until complete solution thereof is effected and the mass 40 becomes clear.

5. The method of treating sheets of cellulosic material to stiffen and render the same fire-proof which consists in heating a suitable volume of water to a temperature of 45 from one hundred and eighty to two hundred degrees Fahrenheit, dissolving sodium carbonate therein, thereafter introducing sodium silicate into the solution thus formed and dissolving the same therein, thereafter 50 introducing tungstate of soda into the last named solution and stirring the mass until complete solution is effected, thereafter placing the composition thus formed in a suitable container and maintaining the same at a 55 temperature of about one hundred and ninety degrees Fahrenheit and submerging a sheet of said cellulosic material therein for a short period of time.

In testimony that I claim the foregoing as 60 my invention, I have hereunto subscribed my name this 30th day of December, A. D., 1924.

CHARLES R. FELIX.

#### CERTIFICATE OF CORRECTION.

Patent No. 1,643,116.

Granted September 20, 1927, to

CHARLES R. FELIX.

It is hereby certified that error appears in the printed specification of the above numbered patent requiring correction as follows: Page 1, line 8, for the misspelled word "desireable" read "desirable"; page 2, line 44, for the word "compound" read "composition"; page 3, line 13, claim 3, after the word "to" insert the word "two"; same page, lines 42 and 43, claim 5, for the misspelled word "cellulostic" read "cellulosic"; and that the said Letters Patent should be read with these corrections therein that the same may conform to the record of the case in the Patent Office.

Signed and sealed this 20th day of December, A. D. 1927.

Seal.

M. J. Moore,  
Acting Commissioner of Patents.